

Dec. 29, 1925.

1,567,091

F. J. TONE

ANTISLIP TILE

Filed Jan. 25, 1922



INVENTOR

Frank J. Tone  
By Bynes, Stellino & Krembs  
his attorneys.

## UNITED STATES PATENT OFFICE.

FRANK J. TONE, OF NIAGARA FALLS, NEW YORK, ASSIGNOR TO THE CARBORUNDUM COMPANY, OF NIAGARA FALLS, NEW YORK, A CORPORATION OF PENNSYLVANIA.

## ANTISLIP TILE.

Application filed January 25, 1922. Serial No. 531,771.

*To all whom it may concern:*

Be it known that I, FRANK J. TONE, a citizen of the United States, residing at Niagara Falls, in the county of Niagara and

5 State of New York, have invented a new and useful Improvement in Antislip Tiles, of which the following is a full, clear, and exact description.

10 My invention relates to tiles, particularly those for floor surfaces, and is designed to provide an improved type of tile which overcomes disadvantages heretofore present in the use of abrasives for giving a non-slip surface.

15 To that end, my invention consists in forming a molded, shaped and preferably burned tile, a certain percentage of the tile mixture being formed of fragments, which fragments are formed by crushing or breaking up a block formed of bonded together abrasive granules or grains. By using these fragments or broken up particles of bonded grains, I have discovered that the grains are firmly retained in place in the tile and 20 do not wear smooth and lose their non-slip properties. Such tiles may also be made in various colors, especially light colors, thus giving advantages in color effects.

25 I will now describe a specific example of my invention.

One embodiment of my invention is illustrated in the accompanying drawing, in which the figure shows a perspective view of a tile of block embodying the present invention.

30 In the drawing, 2 designates a suitable burned tile, slab or block of any desired shape having a tread face 3 in which are clusters of abrasive grains 4 bonded by a ceramic binder as hereinafter described.

35 A mixture is made of aluminous abrasive grains 76 parts, powdered feldspar 18 parts, and powdered kaolin 6 parts. In using the grit or abrasive, I preferably employ several sizes, the coarsest of which may be No. 60 and the finest 150. This mixture is moistened with water and then pressed or otherwise molded into blocks or pieces of a size convenient for subsequent crushing or 40 breaking up. The blocks are then preferably dried and burned in a ceramic kiln at a temperature of about 1350° C. When re-

5 moved from the kiln, the blocks are crushed into fragments which preferably range in size from  $\frac{1}{16}$  to  $\frac{1}{4}$  of an inch in thickness.

I then make up a tile mixture of these bonded abrasive fragments, which may be as follows:

|                              | Parts. |
|------------------------------|--------|
| Abrasive fragments           | 25 60  |
| Feldspar                     | 20     |
| Primary kaolin               | 11     |
| Secondary kaolin             | 11     |
| Ball clay                    | 15     |
| Flint                        | 12 65  |
| Silica sand of about 30 mesh | 6      |

This mixture is then preferably moistened with water to the consistency required for dry pressing, and is then pressed into the form of tiles or tread pieces in ordinary tile 70 presses. The tiles thus formed are then dried and burned, the burning preferably being carried out in a ceramic kiln at a temperature of about 1350° C.

The advantages of my invention result 75 from the use of the bonded abrasive grain fragments in a tile, since the desired non-slip qualities are afforded; the color may be varied widely and light colors used; and the non-slip properties are retained in usage.

It will be understood that while the above is one example of my invention, the abrasive employed and both mixtures may be varied, as well as the method of making the blocks and tiles therefrom.

I claim:

1. As a new article of manufacture, a burned tile having in its tread surface clusters of abrasive grains previously bonded by a ceramic binder.

2. As a new article of manufacture, a burned tile having in its tread surface clusters of abrasive grains previously bonded by a fired ceramic binder.

3. As a new article of manufacture, a burned tile having in its tread surface clusters of abrasive grains previously bonded by a fired ceramic binder, the major portion of the total mass of the clusters being constituted of abrasive grains.

In testimony whereof I have hereunto set my hand.

FRANK J. TONE.